

E. BORMAN.

METHOD OF FILLING HOLES IN METAL PARTS.

APPLICATION FILED MAR. 6, 1917.

1,270,757.

Patented June 25, 1918.

Fig. 1.



Fig. 2.



Fig. 3.



Witness:  
R. L. Fanning

Inventor,  
Emil Borman,  
By - Glenn S. Noble,  
Attly.

# UNITED STATES PATENT OFFICE.

EMIL BORMAN, OF CHICAGO, ILLINOIS.

## METHOD OF FILLING HOLES IN METAL PARTS.

1,270,757.

Specification of Letters Patent. Patented June 25, 1918.

Application filed March 6, 1917. Serial No. 152,682.

To all whom it may concern:

Be it known that I, EMIL BORMAN, a subject of the Czar of Russia, residing at Chicago, in the county of Cook and State of Illinois, have invented or discovered a new and useful Method of Filling Holes in Metal Parts, of which the following is a specification.

Metal castings are frequently defective on account of having sand holes or blow holes therein. Frequently these defects do not appear until the casting has been machined, and a large amount of labor expended thereon. It is often desirable to fill up holes in castings or cylinders or the like in order to change the form of the same. Engine cylinders frequently become scored, and if these scores can be properly filled it avoids the necessity of boring out a cylinder and providing new pistons and rings. The present invention relates to means for filling in such holes and defects or scores with material of such hardness and relatively high melting point that the repaired article will be as good or substantially as good as when new or as though no defect had appeared therein. This invention is particularly applicable to repairing scored or defective cylinders of internal combustion engines, where there is a high degree of temperature and the parts are subjected to considerable wear.

The objects of the present invention or discovery are to provide a new and useful method of repairing metal parts by filling holes with suitable metal so that the repaired part will be as good or substantially as good as when in its original condition; to provide a method for repairing metal parts which includes a novel way of preparing holes or recesses and then filling the holes or recesses with a comparatively hard metal or compound; to provide a method of repairing engine cylinders or like articles, having such advantages as will appear more fully from the following description.

In the accompanying drawings illustrating this invention:

Figure 1 represents a metal part, such for instance as an engine cylinder, having different kinds of defects or injuries to be repaired;

Fig. 2 is a cross sectional view on an enlarged scale, taken on the line 2—2, showing the defects after having been filled;

Fig. 3 is a view similar to Fig. 2, showing the cylinder with the repaired parts ma-

chined or finished to correspond with the internal wall of the cylinder.

While my improved invention or discovery is adapted for filling various kinds of holes or recesses in metal parts, these drawings are illustrative of several repairs or corrections that may be made in accordance therewith. As illustrated in the drawing, 5 indicates a defect such as a sand hole, 65 which only extends partially into the wall; 6 represents a defect such as a blow hole; and 7 represents a defect such as a score made in any well-known manner.

In repairing any of such defects, the hole 70 or recess is first thoroughly cleaned of any loose dirt and is then prepared for filling by applying a cleaning liquid thereto, which thoroughly frees the walls of the opening from grease and the like and prepares the 75 walls of the opening so that the filling material will adhere thereto. For this purpose I prefer to use a compound or liquid made in the following manner: A given amount of zinc is dissolved or treated with 80 approximately double the amount of muriatic or hydrochloric acid. This solution is then mixed with a relatively large volume of nitric acid and water, for instance in the following proportion: ten per cent. of the 85 solution, and forty-five per cent. each of nitric acid and water. It will be observed that these percentages may be varied without departing from the usefulness of the cleaning fluid, and other compounds or acids 90 may be utilized for cleaning different kinds of metals if desired, the former being particularly applicable to cleaning cast iron. After this liquid has been applied to the walls of the part to be repaired, it is left for 95 about five minutes and then the filling compound is inserted in a molten condition. The filling compound which I have preferred to use for filling holes in cast iron consists of the following: ten (10) per cent. 100 of solder composed of tin and lead, twenty-nine per cent. of bismuth, twenty-six per cent. of cobalt, and thirty-five per cent. of zinc. The elements and proportions in this compound may of course be changed or varied to suit different conditions, but I have found that these metals combined in the proportions given form a compound which may be readily applied to the defective part and which will adhere to the prepared walls 110 of the hole in cast iron so as to make a substantially permanent repair. Furthermore,

this compound will be substantially hard and will have a sufficiently high fusing point so that it is particularly applicable for internal combustion engine cylinders, even where very high temperatures are encountered, as in motorcycle engines. This compound is applied in a molten condition to the holes or openings, being poured therein to form fillings 8, 9 and 10, as indicated in Fig. 2. As soon as the compound is placed in position in the hole or recess, sufficient heat is applied thereto to keep the compound in a nearly molten condition and to heat the adjacent walls of the cylinder 11 or part being repaired. This heat may be applied in any desired manner, as by applying a heated iron or the like. It is kept in this heated condition with the compound heated nearly to the melting point for about three to five minutes, and then allowed to cool. A sufficient amount of metal is applied so that it projects outwardly from the surface, for instance as indicated in Fig. 2, so as to insure the complete filling of the hole or score. After this is done the filling is bored, machined or scraped away to leave a surface conforming to the surface of the cylinder or other part which is being treated, as indicated in Fig. 3, which shows the finished article. I have found that by using the particular cleaning compound above set forth, with the zinc dissolved therein, and then applying the filling compound made in the proportions above set forth, makes an exceedingly substantial patch or repair which is not affected by any ordinary temperatures

which are apt to be encountered, and the filling will remain in position even if the hole or scratch to be repaired is exceedingly shallow. It is possible that the cleaning liquid leaves the walls of the hole with a certain amount of zinc embedded or attached to the molecules of the metal forming the wall, so that when the molten compound is applied it will adhere or coalesce with the walls. In any event, the results obtained are as above set forth and the patch or repair will be sufficiently hard so that it is nearly as hard as the walls of the casting. In removing the excess material I have found it advisable to use a tool formed of metal somewhat harder than the compound but not as hard as the walls of the cylinder, so that the machining, scraping or finishing tool will remove the excess compound without scratching the walls of the cylinder.

Having thus described my invention or discovery, which however I do not wish to limit to the exact proportions or compounds herein set forth, what I claim and desire to secure by Letters Patent is:

The process described which consists in treating scores or recesses in a cylinder or the like to a liquid comprising dilute nitric and hydrochloric acids with zinc dissolved therein, filling the score or recess with tin, lead, bismuth, cobalt and zinc, then heating the filling and adjacent walls of the cylinder, and finally removing the excess filling material.

EMIL BORMAN.